

## UNITED STATES PATENT OFFICE

2,378,265

## COLOR PHOTOGRAPHY

Paul W. Vittum and Edwin E. Jelley, Rochester,  
N. Y., assignors to Eastman Kodak Company,  
Rochester, N. Y., a corporation of New Jersey

No Drawing. Application November 29, 1941, Serial No. 421,042. In Great Britain January 17, 1941

5 Claims. (Cl. 95—88)

This invention relates to improvements in photographic processing solutions and particularly to solutions designed for removal of metallic silver from photographic layers.

It is known that in many processes of color photography, both dye images and silver images may be formed in a photographic layer. It is desirable to remove the metallic silver at the end of the process so that a pure transparent dye image remains in the photographic layer. This is generally accomplished by the use of a silver removing bath containing an oxidizing agent for the silver and at the same time or in a subsequent bath dissolving the silver salt thus formed. Silver oxidizing agents ordinarily used are potassium ferricyanide or acid dichromate bleaches followed by a silver halide solvent such as hypo.

It has been found that in some cases the dye or other agents present in the photographic layer tend to occlude the metallic silver and prevent its being acted upon by the oxidizing agents intended to convert it to a silver salt prior to removal. This is especially true in the case of emulsions containing an organic solvent for couplers and dyes such as those described in Mannes & Godowsky U. S. Patent 2,304,940, granted December 15, 1942 and Jelley and Vittum U. S. Patent 2,322,027, granted June 15, 1943. In those processes the coupler originally present in the emulsion layer and the dye formed from it are dissolved in globules of a solvent such as hydrolyzed cellulose acetate or tricresyl phosphate which presumably wets the metallic silver as it is formed and then encloses portions of it which can no longer be affected by aqueous solutions of silver oxidizing agents.

It is, therefore, an object of the present invention to provide novel solutions designed for the removal of metallic silver from photographic layers. A further object is to provide a means for the complete removal of metallic silver from emulsion layers containing dyes protected by organic solvents. Other objects will appear from the following description of our invention.

These objects are accomplished by incorporating in the bleach bath which converts metallic silver to a silver salt, an organic solvent such as a monohydroxy alcohol or an aliphatic ketone. These solvents permit the bleach bath to penetrate any organic material in the emulsion so that the bleach bath is able to act on the metallic silver therein.

As stated above, the bleach baths ordinarily used for the oxidation of metallic silver and conversion of it to a silver salt prior to removal in a

silver salt solvent include compounds such as potassium ferricyanide and acid dichromate. To these bleach baths, we add suitable organic solvents in the proper amount. Organic solvents suitable for use according to our invention include monohydroxy alcohols such as benzyl alcohol, isopropyl alcohol, butyl alcohol,  $\beta$ -phenylethyl alcohol,  $\gamma$ -phenyl-n-propyl alcohol  $\beta$ -and  $\gamma$ -diethylaminopropyl alcohol,  $\beta$ -diethylaminomethyl alcohol, nitroethyl and nitropropyl alcohol, furfuryl alcohol, and tetra-hydrofurfuryl alcohol, and aliphatic ketones such as acetone.

These organic solvents may be used in the bleach bath in quantities ranging from about 1% to about 10% of the volume of the bleach solution. For example, benzyl alcohol may be dissolved in the solution to the extent of about 1%, isopropyl alcohol to the extent of 5 to 10% and acetone to the extent of about 5 to 10%. Acetone is preferred for use in acid dichromate bleaches and the alcohols such as benzyl alcohol appear to give the best results in potassium ferricyanide bleaches.

The following examples illustrate bleach baths which may be used according to our invention.

## Example 1

|                                 |       |    |
|---------------------------------|-------|----|
| Chromic acid (10% solution)     | cc    | 10 |
| Hydrobromic acid (41% solution) | cc    | 3  |
| 30 Potassium bromide            | grams | 2  |
| Acetone                         | cc    | 8  |
| Water to                        | liter | 1  |

## Example 2

|                                   |       |     |
|-----------------------------------|-------|-----|
| 35 Potassium ferricyanide         | grams | 50  |
| Ammonium hydroxide (28% solution) | cc    | 2.5 |
| Potassium bromide                 | grams | 5   |
| Benzyl alcohol                    | do    | 1   |
| Water to                          | liter | 1   |

40 These solutions are followed in each case by the customary solution of hypo or other silver salt solvent such as ammonia, potassium thiocyanate or potassium cyanide.

Our invention is especially useful with methods 45 of color photography such as those described in the Mannes & Godowsky U. S. Patent 2,304,940 and the Jelley and Vittum U. S. Patent 2,322,027, referred to above. Those applications describe processes of color photography in which discrete particles of a color coupler and an organic solvent for the coupler and for the dye formed therefrom are dispersed in a sensitive silver halide emulsion layer. In some cases the organic solvent used to dissolve the coupler and the dye formed from it causes the metallic silver to be retained in the

photographic layer presumably because it wets the metallic silver and prevents action on the metallic silver by the silver oxidizing baths. The silver thus retained causes a degradation of the color image and an improvement in color purity is effected by the use of our invention.

Our invention is also useful in other methods of color photography such as that described in Mannes, Godowsky & Wilder U. S. Patent 2,252,718, August 19, 1941, and in bleach-out methods of color photography, such as that described in Seymour U. S. Patent No. 2,184,022, December 19, 1939.

It will be understood that the modification and examples included herein are illustrative only and that our invention is to be taken as limited only by the scope of the appended claims.

We claim:

1. The method of removing silver from a photographic layer containing silver and dye in particles of water-permeable solvent insoluble in water above 20° C., which comprises oxidizing the silver contained in said solvent to a silver salt in the presence of an organic solvent selected from the group consisting of monohydroxy alcohols and aliphatic ketones, which are soluble in said water-insoluble solvent and removing the silver salt thus formed with a silver salt solvent.

2. The method of removing the silver image from a photographic gelatin layer containing said image associated with dispersed particles of a water-permeable organic compound insoluble in water above 20° C., which comprises converting said silver to a silver salt with a solution of a silver oxidizing agent and an organic solvent for said water-insoluble organic compound, said or-

ganic solvent being selected from the group consisting of monohydroxy alcohols and aliphatic ketones, and removing the silver salt thus formed with a silver salt solvent.

3. The method of removing the silver image from a photographic gelatin layer containing said image associated with dispersed particles of a water-permeable organic compound insoluble in water above 20° C., which comprises converting said silver to a silver salt with a solution of a silver oxidizing agent and a monohydroxy alcohol which is a solvent for said water-insoluble organic compound, and removing the silver salt thus formed with a silver salt solvent.

10 4. The method of removing the silver image from a photographic gelatin layer containing said image associated with dispersed particles of a water-permeable organic compound insoluble in water above 20° C., which comprises converting said silver to a silver salt with a solution of a silver oxidizing agent and an aliphatic ketone which is a solvent for said water-insoluble organic compound, and removing the silver salt thus formed with a silver salt solvent.

20 5. The method of removing the silver image from a photographic gelatin layer containing said image associated with dispersed particles of a water-permeable organic compound insoluble in water above 20° C., which comprises converting said silver to a silver salt with a solution of potassium ferricyanide and a monohydroxy alcohol which is a solvent for said water-insoluble organic compound, and removing the silver salt thus formed with a silver salt solvent.

30 35 PAUL W. VITTM.  
EDWIN E. JELLEY.